

No. 810,933.

PATENTED JAN. 30, 1906.

G. GOLDMAN.  
FABRIC CONTAINING HAIRCLOTH.  
APPLICATION FILED DEO. 4, 1903.

FIG. 1.



FIG. 2.



FIG. 3.



FIG. 4.



FIG. 5.



Witnesses

Chas. T. Davis.

Gustave R. Thompson

Gustave Goldman Inventor

by  
Maurice Cameron Lewis & Macie

Attorneys

# UNITED STATES PATENT OFFICE.

GUSTAV GOLDMAN, OF BALTIMORE, MARYLAND.

## FABRIC CONTAINING HAIRCLOTH.

No. 810,983.

Specification of Letters Patent.

Patented Jan. 30, 1906.

Application filed December 4, 1903. Serial No. 183,823.

*To all whom it may concern:*

Be it known that I, GUSTAV GOLDMAN, of Baltimore, Maryland, have invented a new and useful Fabric Containing Haircloth, which invention is fully set forth in the following specification.

Heretofore haircloth has been employed in a great variety of ways for stiffening garments and like uses, and while it has been found more or less efficient for the purposes for which it was used it is open to a number of serious objections, among which may be mentioned its high cost, the liability of the ends of the hair in the cloth to protrude through the garment, and the necessity of resorting to bindings, tapes, &c., to hold the elastic haircloth in the desired shape and the skill requisite to apply these parts so as to secure the desired or the best results.

The object of the present invention is to provide a product which shall cost less than haircloth as now employed, be free from the objections incident to haircloth, and in addition shall possess certain desirable qualities not found in any haircloth now on the market.

With these objects in view the invention consists in a fabric composed of a body of fibers bound together in a coherent matted or felted mass with a sheet of haircloth incorporated therewith. The haircloth employed may be one in which both the weft and the warp are of hair, or one of these may be hair and the other of cotton or other suitable fiber, as desired, though the latter is preferred because of its greater cheapness. In fact, with this invention in the great majority of cases the amount of hair entering into the haircloth may be much less than what has heretofore been employed in the cheapest grades of such cloth, and as the hair is the expensive factor in the manufacture of haircloth this saving in the amount of hair employed (which may be as great as fifty per cent.) reduces the cost of the fabric which is the subject of the present invention much below that of haircloth, while at the same time producing a greatly superior fabric. The matted or felted mass may be of animal, vegetable, or mineral fibers or mixtures of these, and they are so disposed as to form a sheet of the matted or felted fibers with the haircloth incorporated therein, the whole being so united as to form a compact coherent mass or sheet. In some instances the fibers are disposed so as to form a considerable

body or matted mass of fibers on both sides of the haircloth, the latter being preferably formed with large open meshes through which the fibers from the opposite sides project and intermingle and are firmly united or bound together in the manner hereinafter described or in any other suitable way. It is not essential, however, that there should be a thick mass of the fibers on both sides of the haircloth, as such mass may be upon one side only with the ends of the fibers projecting through the meshes of the cloth and united or bound to each other and to the haircloth. While in most cases the fibers will project through the meshes of the haircloth, it is not essential that this should be the case, as in some instances and with some kinds of fibers the finished fabric is made without the fibers passing through the haircloth to any great extent. Any suitable method may be employed to unite the fibers to each other and to the haircloth. For example, a layer or film of fibers in a loose fluffy condition may have a sheet of haircloth laid thereon and a second layer of fibers in like loose fluffy condition may then be laid over the haircloth and the fibers be then united to each other and to the haircloth by any suitable binding agent, as a sizing, or if the fibers are of a character which will permit of a felting action they may be felted in the usual or any desired way, thereby forming a sheet of felt with the haircloth incorporated therein. One method which has been found to be effective consists in laying down a thin film of the desired fibers in a light fluffy condition, as the same come from the doffer of a carding-machine, for example, and a binder of sizing or a resinate, as zinc resinate, in a dry finely-divided form is then dusted between and upon the fibers, after which the sheet or layer of haircloth is laid upon the film of fibers and more of the binder is then dusted thereon. A second film of the fibers is then laid upon the haircloth and the dry finely-divided binder is dusted between and upon the fibers thereof and the whole then treated so as to convert the dry finely-divided binding material into an active binding agent, whereby the fibers are united to each other and to the haircloth, so that the whole constitutes a matted mass of fibers effectively bound together with the haircloth incorporated therein. The particular procedure for converting the dry finely-divided binding material into an active binding agent will vary somewhat with the nature of the

binder employed. Thus if sizing is used as the binding agent some solvent, as moisture, preferably in the form of steam, is introduced and the whole is then preferably treated by heat and pressure, as by subjecting the fibrous films with the haircloth therebetween to the action of heated rollers. A convenient means of supplying the moisture, heat, and pressure consists in placing the mass of fibers with the haircloth and the dry binding material between moisture-carrying belts and then passing the whole between heated rollers. The heat of the rollers converts the moisture of the belts into steam, which penetrates the fibrous mass, thereby supplying the moisture necessary as a solvent if sizing or its equivalent be used or the fusing heat requisite to convert the resinate or equivalent, if such be used, into an active binding agent.

20 When the sheet has issued from between the heated rollers, it will be found that the fibers composing the two films or layers have been united to each other and to the haircloth, so as to form a matted or felted mass with a

25 sheet of haircloth incorporated therein.

As indicated above, the two films of fibers with the haircloth therebetween may be treated by the usual or any suitable felting process instead of pursuing the method first described. Thus they may be subjected to a rubbing process in the presence of a suitable binder, as a soluble soap, and then passing through a fixing solution, as an alum solution, after which the whole is again rubbed in a flat form in the presence of heat and pressure. This latter method can only be pursued when the fibrous mass is either in whole or in part composed of animal fibers, since vegetable or mineral fibers alone will not

30 "felt." The binder which is employed in either of the processes mentioned serves also as a stiffener, which will cause the completed fabric to retain any shape into which it may be pressed.

45 It will be observed that the fabric herein

described is not a layer of woven fabric with a layer of loose fibers secured by sizing or otherwise on one or both sides thereof, but is a compact mass of fibers united as a whole and having a layer of haircloth incorporated 50 therein or secured thereto.

In the accompanying drawings, which illustrate the invention, are shown, in Figure 1, a cross-section, and in Fig. 2 a plan, of the two fibrous films with the haircloth 55 between them, the fibers being in the loose fluffy condition before they have been treated to unite them into a matted or felted mass; and Fig. 3 is a cross-section of the finished fabric with the matted mass on both sides 60 of the haircloth. Fig. 4 is a cross-section showing the mass of loose fluffy fibers on but one side of the haircloth, and Fig. 5 is a view of Fig. 4 after the same has been treated to form the completed fabric.

In said figures, 1 is the lower, and 2 the upper, film or layer of fibers, and 3 is the sheet of haircloth between said films. In Figs. 4 and 5 the haircloth is laid upon the fibrous layer 1 and the upper layer 2 is omitted.

While processes of making the fabric herein claimed have been described above, such processes are not claimed in the present application, as they form the subject-matter of two other applications of even date herewith.

Having thus described the invention, what is claimed is—

A sheet of haircloth combined with a mass of matted or felted fibers some of which project through the meshes of the cloth, and a 80 waterproof binder uniting the haircloth and fibers together.

In testimony whereof I have signed this specification in the presence of two subscribing witnesses.

GUSTAV GOLDMAN.

Witnesses:

ARTHUR LEE BROWNE,  
FRANCIS T. HOMER.